

## UNITED STATES PATENT OFFICE

2,548,347

## FUEL OIL COMPOSITION

John B. R. Caron, North Plainfield, and Everett B. Glendenning, Cranford, N. J., and Calmy Wies, New York, N. Y., assignors to Shell Development Company, San Francisco, Calif., a corporation of Delaware

No Drawing. Application July 6, 1948  
Serial No. 37,306

20 Claims. (Cl. 44—70)

1

This invention pertains to improvement in hydrocarbon fuels and more particularly to fuel oil compositions capable of preventing or inhibiting the sludging and/or clogging tendencies generally exhibited by hydrocarbon fuels, such as those utilized in burner systems, tanks, diesel and combustion engines, and various other industrial and domestic equipment. In addition, this invention relates to fuel oil compositions capable of removing preformed deleterious matter from filters, screens, and the like, caused by deterioration and/or the presence of foreign bodies (e. g. water) in fuel oils.

Hydrocarbons, such as distillate fuels, for example, those having a normal distillation range of from about 300° F. to about 750° F. and particularly those fuels having a distillation of from about 340° F. to about 640° F., generally have a marked tendency to deteriorate under oxidizing conditions, and to form sludge. Also, the presence of impurities in such fuels, such as the presence of moisture, dispersed water, organic and/or inorganic foreign matter, and the like, causes the formation of insoluble products which tend to settle out and adhere to surfaces with which they come in contact, thereby in turn, causing clogging or plugging of filters, strainers, screens, conduit lines, and the like, of the equipment in which they are used. This necessitates frequent cleaning and even replacement of parts, thereby markedly decreasing the performance efficiency of various equipment which utilizes such fuel oils.

The problem of screen clogging is common, particularly in domestic fuel oil systems employing distillate fuel oils produced by distilling or cracking of petroleum, which fuels, are characterized by their relatively low viscosity and other properties. Fuel oils of this type generally conform to the specifications set forth in Commercial Standards C. S. 12-40 for Nos. 1, 2, and 3, Fuel Oils. Petroleum distillates within the ranges specified and which generally do not exceed 750° F. and preferably are below 675° F. for use as diesel fuels are further examples of the type of oils which under conditions described have a tendency towards screen or filter clogging, particularly when they contain minor amounts of water dispersed therein.

Another place where screen clogging and plugging of conduit lines is encountered is in storage tanks for fuel oils, which tanks may be connected to the burner systems or engines, etc. The stored fuel generally comes in contact with air, moisture, water, etc., which causes forma-

2

tion and precipitation of sludge materials which, in turn, deposit on and clog the screens or filters used for protecting the burners or engines which use such oils as the fuel.

It is an object of this invention to inhibit sludging tendencies of hydrocarbon fuel oils. It is another object of this invention to inhibit sludging and precipitation of contaminants in hydrocarbon distillate fuel oils and particularly in cracked hydrocarbon fuels. It is still another object of this invention to provide distillate fuel oils and particularly fuel oils obtained during cracking of hydrocarbons, which have excellent performance characteristics with respect to freedom from screen clogging, even after extensive storage under oxidizing conditions and in the presence of water. Still another object of this invention is to provide a distillate fuel oil composition which is effective in removing preformed sludge deposits formed in fuel oil systems. Still another object of this invention is to provide a particular type of distillate fuel oil composition, and blends thereof, which are non-corrosive and stable, and which are effective for cleaning and sludge removing.

The above and other objects of this invention may be attained by dispersing, admixing or dissolving in hydrocarbon fuel oils (which normally have a tendency to cause clogging or plugging of screens, filters, conduit lines and the like), a minor amount, which amount is sufficient to inhibit said tendencies, of a partial ester of a polyhydric alcohol, said esters containing one and preferably more than one free hydroxy groups; these partial esters may be considered as acting as surface active agents. If desired, a minor amount of a detergent and/or solutizer may also be added to the composition.

The hydrocarbon distillate fuel oils in which the active ingredient and/or ingredients of this invention are dispersed or dissolved may be treated or untreated catalytically cracked fuel oils, or mixtures or cracked fuels with straight run fuel oils, having components normally distilling from about 300° F. to about 750° F. Generally such fuels of the type under discussion have a boiling range of from about 340° F. to about 700° F. and preferably a boiling range of from about 400° F. to about 675° F.

Cracked fuels may be obtained by thermal or catalytic cracking of certain petroleum hydrocarbon feed stocks. Both the cracked fuels, as well as blends of cracked and straight run fuels, may be acid or caustically treated to improve their stability. Specifically, hydrocarbon dis-

tillates which are utilized as bases in compositions of this invention are cracked gas oils, fuel oils, furnace oils, burner oils, diesel fuel oils, kerosene, etc., and mixtures of said cracked fuels with the corresponding or like straight run hydrocarbon fractions, e. g. fuel oils, etc.

Fuel oils which have marked tendencies towards sludging and clogging of screens, filters, etc., are primarily cracked or blends of cracked and straight run fuel oils which may have the following properties:

|                                       |          |
|---------------------------------------|----------|
| Gravity, °API                         | 29-35    |
| ASTM dist., °F.:                      |          |
| IBP                                   | 400-500  |
| EBP                                   | 600-700  |
| Sulfur, per cent W                    | 0.5-1.05 |
| Carbon residue (10% Btms.) per cent W | 0.1-0.4  |
| Pour point, °F.                       | 0-15     |

The surface active agents which possess the unique property of inhibiting sludge formation or removing performed deposits from surfaces, thereby preventing clogging of systems utilizing fuels normally susceptible to such deterioration are partial esters of polyhydric alcohols and/or modified partial esters of polyhydric alcohols.

One group of esters which is useful as anti-clogging agents in fuel oil compositions may be derived from polyhydric alcohols such as glycerine, glycol, glycol-ethers and their polymerization products such as the polyglycols and polyglycerines. Other polyhydric alcohols which may be used to form the esters are erythritol, pentaerythritol, sorbitol, mannitol, dulcitol, etc.

The acid components of the partial esters may be aliphatic carboxylic acids, e. g. capric, lauric, stearic, oleic acids; fatty acids derived from natural fats and oils; cyclic carboxylic acids, e. g. naphthenic acids; aromatic carboxylic acids, alkyl aromatic carboxylic acids, aralkyl carboxylic acids, e. g. benzoic, salicylic, alkyl salicylic, phthalic, phenyl-acetic, phenyl-stearic, phenyl-oleic acids, rosin acids; sulfonic acids, such as petroleum sulfonic acids, alkyl or aryl sulfonic acids; phosphoric, phosphonic, phosphinic acids and the like. The acids may contain various substituent groups such as branch chains, polar groups such as hydroxy, hydrosulfide, halo, amino groups and the like.

Specific esters of this group may be glyceryl mono-oleate, glyceryl monostearate, glyceryl monoricinoleate, pentaerythritol monolaurate, pentaerythritol mono and dioleate, pentaerythritol monocaprylate, mono, di, and triethylene glycol mono-oleate, propylene glycol monoricinoleate, monoethylene glycol mono-oleate, triethylene glycol monostearate, sorbitol monolaurate, mannitol mono-oleate, mannitol dioleate, sorbitol dioleate, etc.

Another group of partial esters of polyhydric alcohols may be obtained from partially dehydrated polyhydric alcohols. Partial dehydration converts such an alcohol to an inner ether type of compound having hydroxy groups. Specific examples of the polyhydric alcohols which may be dehydrated and then esterified with a suitable acid or acids are mannitol, sorbitol, dulcitol and the like.

Acids particularly useful for the esterification of the cyclic ether-alcohols are fatty acids containing 8 or more carbon atoms and may be derived from natural fats and oils or pure fatty acids or their mixtures may be used. The free fatty acids may be exemplified by capric, palmitic, oleic, stearic acid or the like. In addition to

the fatty acids other acids as noted above may be used and specifically may be exemplified by naphthenic, sulfonic and salicylic acids.

Esters of this type which are particularly suitable as anti-clogging agents in fuel oil compositions may be prepared by the method described in U. S. Patent 2,322,820. Examples of such esters which must contain at least one and preferably more than one free hydroxy group are sorbitan mono and dioleate, sorbitan mono and dilaurate, mannitan mono and distearate, mannitan mono and dioleate, sorbitan mono and dipalmitate, sorbitan sesquioleate, sorbitan monosulfonate, sorbitan mononaphthenate, mannitan monolaurate, etc.

Still another group of partial esters obtained from polyhydric alcohols which are useful as surface active agents in compositions of this invention, are the cyclic ether-alcohol esters as described above which have been modified by being further reacted with an alkylene oxide or a polyalkylene oxide. Thus a sorbitan mono-oleate may be further modified by treatment with ethylene oxide to form the hydroxy ether of sorbitan mono-oleate. Other modified esters of this type may be the polyoxyalkylene sorbitan mono-stearate, polyoxyalkylene sorbitan mono-oleate, polyoxyalkylene sorbitan monolaurate, polyoxyalkylene sorbitan di and tri-oleate, etc.

The polyhydric alcohol esters such as sorbitol mono-oleate or the like may be also modified by being reacted with an alkylene oxide or polyalkylene oxide to form such esters as polyoxyalkylene sorbitol mono-oleate, mixed oleic-lauric acid ester of polyoxyalkylene sorbitol, oleic ester of polyoxyalkylene mannitol, mixed lauric acid ester of sorbitol polyoxyalkylene ethers and polyglycols, etc.

If desired, and under certain conditions of use, it is preferred to add detergents to compositions of this invention. The function of the detergent agents in compositions of this invention is to act as peptizers and aid in inhibiting or preventing the settling and adhering of impurities and sludge to surfaces and allow any impurities present or formed to pass through the screen or filter system.

Detergents which may be used are alkali, alkaline earth and heavy metals and organic nitrogen base salts of various organic acids. The acidic portion of such detergents may be naphthenic acid, sulfonic acids, aromatic and hydroxy aromatic carboxylic acids, aliphatic acids, said acids containing, if desired, substituent groups, e. g., an amino, hydroxide, mercapto, halo and sulfur groups and the like. Also phenates, alcoholates, carbamates, thiocarbamates, xanthates, etc., may be used.

Particularly preferred class of detergents are the salts of alkyl substituted phenol sulfides or its selenide and/or its telluride equivalent. These phenolic salts may be represented by the general formulas:



wherein M is a metal; R and R' represent at least one alkyl radical attached to the aromatic ring Ar, the total number of carbon atoms in all of

such radicals being at least 5; X is O and/or S; Q is S, Se, or Te and n is an integer of from 1 to 4.

To form the salts of these phenolic compounds they may be treated with such metal compounds as Li, Na, K, Cu, Hg, Fe, Mn, Mg, Ca, Ba, Sr, Pb, Ni, Co, Cr, Sn, Fe, etc. Alkaline earth metals are particularly preferred because of their solubility in hydrocarbons and potent detergent properties.

In addition to the normal salts of phenolic compounds, basic salts may be used and can be represented by the formula



wherein the symbols are the same as referred to in the previous formulas. These basic salts may be formed by reacting the aromatic acidic compounds with more than the amount of metal oxide of hydroxide necessary to form the normal salt.

Some specific compounds as represented by the above formulas are: barium tertiary octyl phenol sulfide and disulfide, barium tertiary amyl phenol sulfide, calcium iso-hexadecyl phenol sulfide, magnesium tertiary amyl phenol sulfide, cobalt tertiary amyl phenol sulfide, barium dodecyl salicylate sulfide, sulfide of the barium salt of the ethyl ester of p-hydroxy dithiobenzoic acid, calcium octyl phenol selenide, etc. The amount of detergent salt used may vary from between about 5 and 15% and preferably is kept below 10%.

Another preferred class of detergents comprises the alkali (e. g. Na, Li, K) and/or alkaline earth metal (e. g. Mg, Ca, Sr, Ba) salts of petroleum sulfonic acids, preferably of high molecule weight, derived from petroleum hydrocarbon crudes and fractions thereof, which are the so-called mixed type i. e. containing naphthenic type hydrocarbons.

These oil-soluble petroleum sulfonates may be obtained by various processes, such as those disclosed in the U. S. patents, 2,388,677, 2,395,713, 2,413,311, 2,414,773, 2,416,397, and if desired, purified by such means as those disclosed in U. S. patents, 2,236,933, 2,334,532, 2,357,866, 2,368,452, and 2,406,753.

The metal salts of the specific type of petroleum sulfonic acid under discussion or other type of detergents may be added to the concentrate or base in amounts of from about 5% to about 15% and preferably below 10%.

In systems wherein substantial amounts of moisture are present a drying agent may be added which is compatible with the active ingredients of this invention. By tying up most of the free moisture in this manner, the amount which would normally combine with sludge forming materials is diminished, thus alleviating a most aggravating clogging problem.

Drying agents which are particularly suited are the glycol-ether type such as diethylene glycol monomethyl, ethyl N- and isopropyl ether, diethylene glycol mono-butyl ether, diethylene glycol mono-decyl ether, etc. also dipropylene glycol mono-ethyl, dipropylene mono-isopropyl ether, dipropylene glycol mono-isoamyl ether, diisobutylene glycol mono-isopropyl ether, ethylene-propylene glycol mono ethyl ether, ethylene-isobutylene glycol mono-isopropyl ether, etc. Instead of the glycol-ethers, various alcohols may be used such as diols having 6 or more carbon atoms in the molecule such as hexylene glycol,

decylene glycol, cetylene glycol, etc. diglycols such as dipropylene glycol, dibutylene glycol, diamylene glycol, ether alcohols and particularly the glycol mono alkyl ethers, e. g., the Cellosolves such as ethylene glycol mono-ethyl ether, ethylene glycol mono-propyl ether, ethylene glycol mono-tert.-butyl ether, propylene glycol mono-butyl ether, propylene glycol mono-ethyl ether, propylene glycol mono-isoamyl ether, etc. Also glycol mono-tert.-butyl ether, ethylene glycol mono-butyl ether, propylene glycol mono-ethyl ether, propylene glycol mono-isoamyl ether, etc. Also glycerine and the like may be used.

The amount of these drying agent materials, when used, constitutes a substantial portion of the base and generally is around about 50% or more. However, under certain conditions these materials may be omitted from the base.

The following is a general formula of a base composition of this invention:

|                                                                                                                         | Per cent |
|-------------------------------------------------------------------------------------------------------------------------|----------|
| Partial ester of a polyhydric alcohol alcohol containing at least one free hydroxy group and/or modified esters thereof | 10-20    |
| Detergent e. g. phenate, sulfonate, etc.                                                                                | 0-10     |
| Drying agent, e. g. glycol ether                                                                                        | 0-50     |
| Hydrocarbon fuel oil                                                                                                    | Balance  |
| Specific base (concentrate) compositions may be illustrated by the following examples:                                  |          |
| Composition A:                                                                                                          |          |
| Sorbitan monolaurate                                                                                                    | 10       |
| Hydrocarbon fuel oil                                                                                                    | 90       |
| Composition B:                                                                                                          |          |
| Mannitan monolaurate                                                                                                    | 10       |
| Hydrocarbon fuel oil                                                                                                    | 90       |
| Composition C:                                                                                                          |          |
| Mixed lauric acid ester of sorbitol poly-oxylalkene ether and polyglycols                                               | 10       |
| Hydrocarbon fuel oil                                                                                                    | 90       |
| Composition D:                                                                                                          |          |
| Polyethylene glycol mono or dioleate                                                                                    | 10       |
| Hydrocarbon fuel oil                                                                                                    | 90       |
| Composition E:                                                                                                          |          |
| Glyceryl monooleate                                                                                                     | 10       |
| Diethylene glycol monobutyl ether                                                                                       | 10       |
| Hydrocarbon fuel oil                                                                                                    | 80       |
| Composition F:                                                                                                          |          |
| Sorbitan monooleate                                                                                                     | 15       |
| Barium salt of alkyl phenol disulfide                                                                                   | 10       |
| Hydrocarbon fuel oil                                                                                                    | Balance  |
| Composition G:                                                                                                          |          |
| Sorbitan monooleate                                                                                                     | 15       |
| Sodium petroleum sulfonate                                                                                              | 15       |
| Barium salt of alkyl phenol disulfide                                                                                   | 5        |
| Hydrocarbon fuel oil                                                                                                    | Balance  |
| Composition H:                                                                                                          |          |
| Sorbitol monooleate                                                                                                     | 10       |
| Sodium petroleum sulfonate                                                                                              | 5        |
| Hydrocarbon fuel oil                                                                                                    | Balance  |
| Composition I:                                                                                                          |          |
| Sorbitan monolaurate                                                                                                    | 10       |
| modified with ethylene oxide                                                                                            | 10       |
| Diethylene glycol monobutyl ether                                                                                       | 20       |
| Hydrocarbon fuel oil                                                                                                    | Balance  |
| Composition J:                                                                                                          |          |
| Sorbitan monolaurate                                                                                                    | 10       |
| modified with ethylene oxide                                                                                            | 10       |
| Sodium petroleum sulfonate                                                                                              | 5        |
| Hydrocarbon fuel oil                                                                                                    | 85       |
| Composition K:                                                                                                          |          |
| Sorbitan sesquioleate                                                                                                   | 10       |
| Hydrocarbon fuel oil                                                                                                    | 90       |

Compositions of this invention are generally mixed in amounts of 1 pint or less with from about 250 to about 1000 gallons of fuel oil. Thus, for example, on a percentage basis of fuel used, one pint of any one of the compositions described above per 250 gallons of fuel would correspond to approximately the following concentration of the active ingredients: Partial ester of a polyhydric alcohol as described, 0.0025 to 0.005%; detergent, 0 to about 0.0025%; drying agent, 0 to about 0.0265%.

To inhibit any corrosive tendencies of fuel compositions of this invention a minute amount of caustic or aromatic nitrogen compound such as aniline may be added. These compounds act as alkaline reserves and render the fuel compositions substantially non-corrosive to copper, brass, and other metals.

The following illustrates the effectiveness of compositions of this invention as sludge inhibitors and anti-clogging agents.

#### Example I

To a number of sample bottles each containing approximately 50 cc. of fuel oil normally susceptible to cause clogging a minute amount of about 0.15 cc. of water was added and also to each sample bottle about 0.05% of a specific base composition as noted in the table below was also added. The bottles were shaken thoroughly and then permitted to stand for about one hour. Suspension properties of water and inert particles were observed and noted after one hour. After one hour of standing the bottles were shaken again and the contents poured into a very fine strainer container. Wetting and drainage properties on the bottle were observed just before and after removal of contents. The time of efflux of the composition was noted for each composition and the condition of the strainer observed.

#### Example II

Another test, the results of which are also tabulated below, in order to determine the effectiveness of compositions of this invention for anti-sludging and clogging properties was conducted in the following manner: About 0.05% of base compositions of this invention was added to fuel oils containing entrained moisture. The samples were allowed to age for two days. These samples were then shaken and evaluated for their anti-clogging properties, as related in the preceding paragraph.

| 0.05% or less base composition as noted in fuel oil containing entrained moisture | Properties evaluated immediately after adding concentrate to fuel oil (Example I) |           |            | Same properties after aging of fuel oil (Example II) |           |            |
|-----------------------------------------------------------------------------------|-----------------------------------------------------------------------------------|-----------|------------|------------------------------------------------------|-----------|------------|
|                                                                                   | Strainer                                                                          | Drainage  | Suspension | Strainer                                             | Drainage  | Suspension |
| Composition A                                                                     | Excellent                                                                         | Excellent | Excellent  | Excellent                                            | Excellent | Excellent  |
| Composition B                                                                     | Good                                                                              | Fair      | Fair       | Fair                                                 | Fair      | Fair       |
| Composition K                                                                     | Excellent                                                                         | Good      | Good       | do                                                   | do        | Do         |
| Composition D                                                                     | do                                                                                | Excellent | Excellent  | Excellent                                            | Excellent | Excellent  |
| Composition J                                                                     | do                                                                                | do        | do         | do                                                   | do        | Do         |
| Composition C                                                                     | do                                                                                | Good      | Good       | do                                                   | do        | Do         |
| Composition F                                                                     | do                                                                                | do        | do         | do                                                   | do        | Do         |
| Composition H                                                                     | do                                                                                | Excellent | Excellent  | do                                                   | do        | Do         |
| Undoped fuel oil                                                                  | Poor                                                                              | Poor      | Poor       | Poor                                                 | Poor      | Poor       |

To compositions of this invention may be added minor amounts of a foaming inhibitor such as silicon liquids, e. g., dimethyl silicone, fluoro organic compounds, fluoro paraffins, salts of alkyl alkylene phosphates and the like. Compositions of this invention may be used to remove deposits, formed on metal surfaces such as in tubes, evapo-

rators, heat exchangers, distillation and cracking equipment and the like. They are non-corrosive and do not interfere with the functioning of the liquid in which dispersed.

It is to be understood that while the features of the invention have been described and illustrated in connection with certain specific examples this invention, however, is not to be limited thereto or otherwise restricted, except by the scope of the appended claims.

We claim as our invention:

1. A fuel oil containing substantial amount of cracked components and entrained moisture and normally susceptible to cause clogging said fuel oil rendered non-clogging by incorporation therein from about 0.0025 to about 0.005% of sorbitan monolaurate.

2. A fuel oil containing substantial amount of cracked components and entrained moisture and normally susceptible to cause clogging said fuel oil rendered non-clogging by incorporation therein from about 0.0025 to about 0.005% of polyoxyalkylene derivative of a partial ester of sorbitan oleate.

3. A fuel oil containing substantial amount of cracked components and entrained moisture and normally susceptible to cause clogging said fuel oil rendered non-clogging by incorporation therein from about 0.0025 to about 0.005% of a partial ester of polyethylene glycol oleate.

4. A fuel oil containing substantial amount of cracked components and entrained moisture and normally susceptible to cause clogging said fuel oil rendered non-clogging by incorporation therein from about 0.0025 to about 0.005% of sorbitan monolaurate and about 0.0025% of barium salt of alkyl phenol disulfide.

5. A fuel oil containing substantial amount of cracked components and entrained moisture and normally susceptible to cause clogging said fuel oil rendered non-clogging by incorporation therein from about 0.0025 to about 0.005% of polyoxyalkylene derivative of a partial ester of sorbitan oleate and about 0.0025% of barium salt of alkyl phenol disulfide.

6. A fuel oil containing substantial amount of cracked components and entrained moisture and normally susceptible to cause clogging said fuel oil rendered non-clogging by incorporation therein from about 0.0025 to about 0.005% of a partial ester of polyethylene glycol oleate and about 0.0025% barium salt of alkyl phenol disulfide.

7. A fuel oil containing substantial amount of

cracked components and entrained moisture and normally susceptible to cause clogging said fuel oil rendered non-clogging by incorporation therein from about 0.0025 to about 0.005% of sorbitan monolaurate and about 0.0025% of alkali metal petroleum sulfonate.

75 8. A fuel oil containing substantial amount of

cracked components and entrained moisture and normally susceptible to cause clogging said fuel oil rendered non-clogging by incorporation therein from about 0.0025 to about 0.005% of polyoxyalkylene derivative of a partial ester of sorbitan oleate and about 0.0025% of alkali metal petroleum sulfonate.

9. A fuel oil containing substantial amount of cracked components and entrained moisture and normally susceptible to cause clogging said fuel oil rendered non-clogging by incorporation therein from about 0.0025 to about 0.005% of a partial ester of polyethylene glycol oleate and about 0.0025% of alkali metal petroleum sulfonate.

10. A fuel oil containing substantial amount of cracked components and entrained moisture and normally susceptible to cause clogging said fuel oil rendered non-clogging by incorporation therein from about 0.0025% to about 0.005% of a partial ester of a polyhydric alcohol, said ester having at least one free hydroxyl group and about 0.0025% of a detergent selected from the class consisting of oil-soluble metal phenate and metal petroleum sulfonate.

11. An anti-clogging concentrate adapted to be added to hydrocarbon fuel oil containing substantial cracked components and normally susceptible to clogging, said concentrate consisting essentially of from 10-20% sorbitan monolaurate and the balance being a fuel oil having a boiling range within the range of from 300 to 750° F. and containing substantial cracked components.

12. An anti-clogging concentrate adapted to be added to hydrocarbon fuel oil containing substantial cracked components and normally susceptible to clogging, said concentrate consisting essentially of from 10-20% polyoxyalkylene derivative of a partial ester of sorbitan and oleic acid and the balance being a liquid hydrocarbon distillate fraction having a boiling range of from 300 to 700° F.

13. An anti-clogging concentrate adapted to be added to hydrocarbon fuel oil containing substantial cracked components and normally susceptible to clogging, said concentrate consisting essentially of from 10-20% sorbitan monolaurate, about 10% barium salt of alkyl phenol sulfide and the balance being a liquid hydrocarbon distillate fraction having a boiling range of from 300 to 700° F.

14. An anti-clogging concentrate adapted to be added to hydrocarbon fuel oil containing substantial cracked components and normally susceptible to clogging, said concentrate consisting essentially of from 10-20% polyoxyalkylene derivative of a partial ester of sorbitan and oleic acid, about 10% barium salt of alkyl phenol sulfide and the balance being a liquid hydrocarbon distillate fraction having a boiling range of from 300 to 700° F.

15. An anti-clogging concentrate adapted to be added to hydrocarbon fuel oil containing substantial cracked components and normally susceptible to clogging, said concentrate consisting essentially of from 10-20% a partial ester of polyethylene glycol and oleic acid and the balance being a liquid hydrocarbon distillate fraction having a boiling range of from 300 to 700° F.

16. An anti-clogging concentrate adapted to be added to hydrocarbon fuel oil containing substantial cracked components and normally susceptible to clogging, said concentrate consisting essentially of from 10-20% of a partial ester of polyethylene glycol and oleic acid, about 10% barium salt of alkyl phenol sulfide and the balance being a liquid hydrocarbon distillate fraction having a boiling range of from 300 to 700° F.

17. An anti-clogging concentrate adapted to be added to hydrocarbon fuel oil containing substantial cracked components and normally susceptible to clogging, said concentrate consisting essentially of from 10-20% sorbitan monolaurate, about 10% alkali metal petroleum sulfonate and the balance being a liquid hydrocarbon distillate fraction having a boiling range of from 300 to 700° F.

18. An anti-clogging concentrate adapted to be added to hydrocarbon fuel oil containing substantial cracked components and normally susceptible to clogging, said concentrate consisting essentially of from 10-20% polyoxyalkylene derivative of a partial ester of sorbitan and oleic acid, about 10% alkali metal petroleum sulfonate and the balance being a liquid hydrocarbon distillate fraction having a boiling range of from 300 to 700° F.

19. An anti-clogging concentrate adapted to be added to hydrocarbon fuel oil containing substantial cracked components and normally susceptible to clogging, said concentrate consisting essentially of from 10-20% partial ester of polyethylene glycol and oleic acid, about 10% alkali metal petroleum sulfonate and the balance being a liquid hydrocarbon distillate fraction having a boiling range of from 300 to 700° F.

20. An anti-clogging concentrate adapted to be added to hydrocarbon fuel oil containing substantial cracked components and normally susceptible to clogging, said concentrate consisting essentially of from 10-20% of a partial ester of a polyhydric alcohol and a fatty acid containing at least 8 carbon atoms and about 10% of a detergent selected from the class consisting of oil-soluble metal phenate and oil-soluble metal petroleum sulfonate and the balance being a liquid hydrocarbon distillate fraction having a boiling range of from 300 to 700° F.

JOHN B. R. CARON.  
EVERETT B. GLENDENNING.  
CALMY WIES.

#### REFERENCES CITED

The following references are of record in the file of this patent:

| UNITED STATES PATENTS |                |                |
|-----------------------|----------------|----------------|
| Number                | Name           | Date           |
| 2,296,069             | Talbert et al. | Sept. 15, 1942 |
| 2,322,820             | Brown          | June 29, 1943  |
| 2,362,291             | Winning        | Nov. 7, 1944   |
| 2,369,490             | Proell         | Feb. 13, 1945  |
| 2,398,193             | Sharp          | Apr. 9, 1946   |
| 2,434,490             | Duncan         | Jan. 13, 1948  |
| 2,456,569             | Smith          | Dec. 14, 1948  |
| 2,482,517             | Schiermeier    | Sept. 20, 1949 |